

Patented Mar. 26, 1929.

1,706,840

# UNITED STATES PATENT OFFICE.

ALBERT L. CLAPP, OF DANVERS, MASSACHUSETTS, ASSIGNOR TO BENNETT, INCORPORATED, OF BOSTON, MASSACHUSETTS, A CORPORATION OF MASSACHUSETTS.

## WATERPROOF PAPER AND PROCESS OF PRODUCING THE SAME.

No Drawing.

Application filed February 27, 1926. Serial No. 91,256.

This invention relates to the preparation of a sized or waterproof paper in which is uniformly incorporated throughout a sizing agent, and more particularly an aluminum or other metallic soap, which has the property of rendering the paper non-absorbent and resistant to the passage of water, ink, and other like aqueous liquids therethrough.

The sizing is usually carried out on the 10 pulp stock in the beater engine, the sizing agent being incorporated into the stock in the form of a soluble soap during or after beating. The sizing is then effected by precipitating or "fixing" the size on the fibers 15 by the addition of aluminum sulphate, alum, or other soluble metallic salts or mixture of salts. This causes the precipitation of an aluminum or other metallic soap in situ on all the fibers, producing a homogeneously 20 sized stock. Paper formed from the sized stock, upon being dried, is non-absorbent and water-resistant.

I have found that straight chain fatty acid soaps, and more especially soaps produced from certain vegetable oils, e. g., linseed, cottonseed, palm, or China wood oils, and certain animal fats, e. g., stearin or olein, when employed for sizing pulp prior to its formation into paper, yield a sticky and tacky aluminum or other metallic soap which renders the stock tacky. Consequ- 25 ently, when such stock is subsequently formed into paper, it gums the wires of a Fourdrinier machine, or the wires of the cylinder 30 mould and felts of a cylinder machine, great difficulty being experienced in maintaining the paper-forming machinery in condition for effective operation. This difficulty accompanying the use of fatty acid soaps in 35 large measure accounts for their heretofore relatively limited use in the sizing of paper.

I have discovered that I may advantageously employ soaps for sizing paper pulp which when used as ordinarily yield sticky 40 and tacky aluminum or other metallic soaps, that render the paper-making stock sticky and tacky. This may be accomplished if the precipitation of the metallic soap on the stock is effected simultaneously with the 45 precipitation of a non-adherent, flocculent precipitate, which envelops or films the sticky metallic soap particles so as to produce a non-sticky sized stock. Such a stock 50 may be run on to the paper machine with- 55 out difficulty.

The soap employed as a sizing agent may be produced as ordinarily by the saponification of olein, palmatin, or other suitable fatty acids or fatty acid esters with caustic soda or other equivalent alkaline compound. 60 The soap is introduced into the pulp in the beater engine, together with a suitable quantity of a soluble reagent such as sodium silicate, which is capable of reacting with aluminum sulphate to yield a voluminous, 65 flocculent precipitate (of aluminum silicate when sodium silicate and aluminum sulphate are used), which serves to envelop or film the aluminum soap particles, thus inhibiting a tackiness of the stock on which 70 they become fixed. The precipitated aluminum silicate also serves as an excellent loading or filling material for the paper. It further serves better to "pull down" and 75 fix the precipitated soap on the fibers, giving a high factor of soap-size retentivity by the stock.

In carrying out the process, I may, for example, proceed about as follows: The beater engine is charged with sulphite pulp 80 and the amount of water necessary to insure its circulation is added. The pulp is then beaten to the extent desired for paper-forming operation, during or after the completion of which the sizing of the stock is 85 effected.

The sizing soap is preferably added to the beater and incorporated into the pulp after the beating has been completed, together with the sodium silicate in the form 90 of an aqueous cream or paste. The aqueous sizing paste is uniformly admixed with the pulp prior to its precipitation in situ on the fibers. The addition of the sizing paste after the beating operation tends to prevent 95 excessive foaming. The paste may contain about 10 to 15 pounds of soap (e. g., sodium stearate or sodium oleate, or a mixture of both) to 1,000 pounds of pulp, and about 15 to 20 pounds of sodium silicate (60° 100 Baumé). The paste may be prepared by dissolving the soap at about 220° to 250° F., in about 100 to 150 pounds of water, and adding sodium silicate to the soap solution thus formed. The paste is preferably allowed to cool prior to the addition to and incorporation in the stock in the beater. The addition of a cooled aqueous paste diminishes the tendency to excessive foaming in the beater. If desired, however, the 110

soap solution and sodium silicate may be separately added and incorporated into the stock in the beater.

After the soap solution and sodium silicate have been uniformly admixed with the pulp, the soap and sodium silicate are caused to react simultaneously by adding a solution of aluminum sulphate, or alum, to the beater engine, thus producing a voluminous mixed 5 or composite precipitate of aluminum soap and aluminum silicate, which becomes fixed on the fibers, about 40 to 50 parts of alum insuring a complete precipitation. The precipitate consists of particles of aluminum 10 soap, protected by a non-sticky film of aluminum silicate, which renders the fibers to which they become fixed non-sticky. While a smaller quantity of sodium silicate may be employed, it is desirable to provide a sufficient 15 amount of aluminum silicate to cover adequately the aluminum soap particles and thus produce a substantially non-adhesive sized stock and much less can not safely be counted upon to produce the desired results.

20 The sized stock may be formed into paper on a Fourdrinier or a cylinder machine, without difficulty. The aluminum silicate, as precipitated, serves as an excellent loading or filling material, and imparts bulk and 25 opaqueness to the paper.

The amount of sodium silicate introduced with the soap in the beater engine may be regulated to produce the filling desired, but, in any event, enough sodium silicate should 30 be added to insure successful paper-forming machine operation. If desired, the fatty acid soap may be replaced in part by rosin size. In such case the quantity of sodium silicate may be correspondingly reduced and 35 thus the amount of filler or loading material in the finished paper present as aluminum silicate may be regulated. Other loading or 40 sizing agents also may be incorporated, together with those agents mentioned.

45 While I have confined myself to a specific example which has been found to yield the desired results for a certain paper product, it should be obvious that the conditions under which the process is carried out, and the 50 proportion of the various agents employed may be changed, depending upon the characteristics desired in the finished paper. For instance, in the preparation of wrapping papers I may employ kraft or sulphate 55 pulp in the stock furnish and use other proportions of sodium silicate and sizing soap. Other pulp furnishes and a suitable proportion of sizing soap and sodium silicate may also be employed.

60 In carrying out the sizing operation it is essential that the precipitation of the aluminum soap be effected simultaneously with the precipitation of the aluminum silicate, but it is not essential that the soap and sodium silicate be added to the stock in the 65

beater engine prior to the aluminum sulphate. Thus I may first add the desired amount of alum to the stock and then add the mixed sodium silicate and soap paste thereto, but better results are obtained by 70 adding the alum subsequent to the incorporation of the sizing paste into the stock.

By the term "soap" as employed in the specification and in the appended claims, unless the context indicates clearly to the 75 contrary, I mean the saponified product of a straight chain fatty acid or fatty acid ester and which is capable of uniting with aluminum sulphate or other soluble metallic salts or mixture of salts to form a water- 80 proof, insoluble, and sticky soap, as distinguished from sodium resinate, which has a ring structure and does not form a sticky soap under the same conditions. Among 85 such soluble metallic salts may be mentioned zinc sulphate, magnesium sulphate and the like. These may be used together with a solution of a suitable flocculating agent, to replace aluminum sulphate. Since there are 90 various metallic soaps which may be produced, e. g., zinc stearate, magnesium resinate, aluminum palmitate and the like, having different characteristics, the characteristics imparted to the paper may be made to vary accordingly, depending upon the particular soap or mixture of soaps in the 95 paper.

I claim:

1. A process of making paper, which comprises incorporating a soluble straight chain fatty acid soap into paper pulp together with sodium silicate, adding metal salt in sufficient quantity to precipitate both the soap and the sodium silicate, and running the pulp off on a paper machine. 100

2. A process of making paper, which comprises incorporating a straight chain fatty acid sodium soap into paper pulp together with sodium silicate, adding alum in sufficient quantity to precipitate both the soap and the sodium silicate, and running the pulp off on a paper machine. 105

3. A process which comprises disseminating sodium stearate together with sodium silicate through cellulose pulp, adding alum in sufficient amount to react with both the sodium stearate and sodium silicate, and running the pulp out on a paper machine. 115

4. A sized and filled paper comprising aluminum stearate and aluminum silicate. 120

5. A sized and filled paper, comprising a straight chain fatty acid metallic soap and a metallic silicate.

6. A sized and filled paper, comprising a straight chain fatty acid aluminum soap and aluminum silicate. 125

In testimony whereof I have affixed my signature.

ALBERT L. CLAPP.